

## UNITED STATES PATENT OFFICE

RUDOLF RIPA, OF FRANKFORT-ON-THE-MAIN, GERMANY, ASSIGNOR TO POMOSIN WERKE G. M. B. H., OF FRANKFORT-ON-THE-MAIN, GERMANY, A COMPANY OF GERMANY

## HARDENING OF STEEL

No Drawing. Application filed April 23, 1931, Serial No. 532,277, and in Germany April 30, 1930.

This invention relates to improvements in the hardening of steel and like metal alloys.

I have ascertained that the heat conductivity of pectin solutions is approximately the same as that of oils, which are particularly suitable for the hardening of steel.

Based on these facts, I have investigated the hardening of steel with pectin solutions and pectin extracts and have found that 10 these exhibit outstanding advantages for this purpose, it being understood that the procedure or manner of using these pectin solutions or extracts is the same as in the case of the oil customarily employed for hardening steel.

Thus it was found possible to obtain varying results, according to the concentration of the pectin solution so that depending upon the concentration of the pectin solution employed, various degrees of hardness, tenacity and brittleness of the hardened steel can be obtained.

The pectin solutions employed according to this invention offer as compared with steel 25 hardening oils, the advantage of accurate adjustability. Oil as is known, is immiscible with water, whereas mixtures of water and pectin can be prepared in any desired proportion.

30 A further advantage is that oil is combustible, while pectin solutions are not. Since the steel is generally introduced (plunged) into the hardening bath in a glowing condition, this fact is of special importance.

35 The most important advantage is, however, the low price of the pectin solutions, which are many times cheaper than hardening oils.

Yet another advantage of the process of 40 the invention is that the hardening and tempering, which have hitherto been effected in two separate operations, can by a suitable regulation of the concentration of the pectin solution be carried out in one operation.

45 For the hardening of steels pectin solutions of 0.5 to 15% and over can be used. Instead of artificial pectin solutions, natural pectin extracts, coming from portions of plants, which can be concentrated or diluted 50 as desired, can be used. When it is desired

to obtain high brittleness and hardness, solutions with small pectin content are used. When, however, a steel of high tenacity and low hardness is desired, higher concentrations are used. The desired hardening effect 55 must be exactly determined by empirical means, depending on the composition of the steel. For example, for tool steel, which should show great hardness, but be as tough as possible, about 4% pectin solution is used. 60

Instead of pectin solutions, solutions of other plant colloids or gelatine, albumen, dextrin, starches, plant gums, agar-agar, tragacanth, gum arabic, alkali cellulose and the like can be used with similar results. I 65 have found that pectin solutions (or extracts, as their equivalents) yield the best results, which fact I attribute partly to the incombustible character of pectin, and partly to the fact that it excels as a poor conductor of heat. 70

What I claim is:—

The process of treating steels and like metal alloys, which consists in plunging them while hot into a hardening pectin solution.

In testimony whereof I hereunto affix my 75 signature this 13th day of April, 1931.

RUDOLF RIPA.

80

85

90

95

100